# EUROPEAN PATENT APPLICATION

(11) **EP 2 479 380 A1**
(43) Date of publication of application: **25.07.2012**
(21) Application number: 12151843.5
(22) Date of filing: 19.01.2012
(51) Int. Cl.: F01D 5/02, F01D 5/06, F01D 5/28

(54) **A welded rotor, a steam turbine having a welded rotor and a method for producing a welded rotor**

(30) Priority: 21.01.2011 US 201113011387
(71) Applicant: General Electric Company, Schenectady, NY 12345 (US)
(72) Inventor: Farineau, Thomas J., Schenectady, NY 12345 (US); Fernandez, Manuel Julio Gomez, 02-256 Warsaw (PL)
(74) Representative: Szary, Anne Catherine

(57) **Abstract**

A welded rotor, a steam turbine having a welded rotor, and a method of producing a welded rotor are disclosed. The welded rotor includes a high pressure section and an intermediate pressure section. The welded rotor includes a shaft having a high temperature material section joined to a first and second low temperature material sections.

## Description

### FIELD OF THE INVENTION

The present invention is generally directed to steam turbines, and more specifically directed to a steam turbine having a welded rotor shaft.

### BACKGROUND OF THE INVENTION

A typical steam turbine plant may be equipped with a high pressure steam turbine, an intermediate pressure steam turbine and a low pressure steam turbine. Each steam turbine is formed of materials appropriate to withstand operating conditions, pressure, temperature, flow rate, etc., for that particular turbine.

Recently, steam turbine plant designs directed toward a larger capacity and a higher efficiency have been designed that include steam turbines that operate over a range of pressures and temperatures. The designs have included high-low pressure integrated, high-intermediate -low pressure integrated, and intermediate-low pressure integrated steam turbine rotors integrated into one piece and using the same metal material for each steam turbine. Often, a metal is used that is capable of performing in the highest of operating conditions for that turbine, thereby increasing the overall cost of the turbine.

A steam turbine conventionally includes a rotor and a casing jacket. The rotor includes a rotatably mounted turbine shaft that includes blades. When heated and pressurized steam flows through the flow space between the casing jacket and the rotor, the turbine shaft is set in rotation as energy is transferred from the steam to the rotor. The rotor, and in particular the rotor shaft, often forms of the bulk of the metal of the turbine. Thus, the metal that forms the rotor significantly contributes to the cost of the turbine. If the rotor is formed of a high cost, high temperature metal, the cost is even further increased.

Accordingly, it would be desirable to provide a steam turbine rotor formed of the least amount of high temperature materials.

### SUMMARY OF THE INVENTION

According to an exemplary embodiment of the present disclosure, a rotor is disclosed that includes a high pressure section having a first end and a second end, and an intermediate pressure section joined to the second end of the high pressure section. The high pressure section includes a high temperature material section formed of a high temperature material. The high pressure section having a first end and a second end opposite thereof. A first low temperature material section formed of a first low temperature material is joined to the first end of the high temperature material section, and a second low temperature material section formed of a second low temperature material is joined to the second end of the high temperature material.

According to another exemplary embodiment of the present disclosure, a steam turbine is disclosed that includes a rotor. The rotor includes a high pressure section having a first end and a second end, and an intermediate pressure section joined to the second end of the high pressure section. The high pressure section includes a high temperature material section formed of a high temperature material and having a first end and a second end opposite thereof, and a first low temperature material section formed of a first low temperature material joined to the first end of the high temperature material section, and a second low temperature material section formed of a second low temperature material joined to the second end of the high temperature material section.

According to another exemplary embodiment of the present disclosure, a method of manufacturing a rotor is disclosed that includes providing a shaft high pressure section, and joining a shaft intermediate pressure section to the shaft high pressure section. The shaft high pressure section includes a first end and a second end, and a first low temperature material section is joined to the first end of the high temperature material section, and a second low temperature material section is joined to the second end of the high temperature material section.

One advantage of an embodiment of the present disclosure includes providing a lower cost steam turbine rotor.

Another advantage of an embodiment of the present disclosure includes providing a lower cost steam turbine rotor that has a reduced amount of high temperature material.

Another advantage of an embodiment of the present disclosure includes providing a lower cost steam turbine.

Another advantage of an embodiment of the present disclosure includes providing a lower cost steam turbine that has a reduced amount of high temperature material.

Another advantage of an embodiment of the present disclosure includes providing a lower cost steam turbine rotor that uses a reduced amount of high temperature material that may not be available in large volumes.

Another advantage of an embodiment of the present disclosure includes providing a lower cost steam turbine rotor that uses smaller ingots of high temperature materials for manufacture.

Other features and advantages of the present invention will be apparent from the following more detailed description of the preferred embodiment, taken in conjunction with the accompanying drawings which illustrate, by way of example, the principles of the invention.

### BRIEF DESCRIPTION OF THE DRAWINGS

Fig. 1 is a sectional view of a steam turbine according to the present disclosure
Fig. 2 is a partial cross-sectional view of an embodiment of a steam turbine rotor according to the invention.
Fig. 3 is a partial cross-sectional view of a portion of the steam turbine of Fig. 1.
Fig. 4 is another partial cross-sectional view of a portion of the steam turbine of Fig. 1.

Fig. 5 is an illustration of another embodiment of a steam turbine according to the present disclosure.

Wherever possible, the same reference numbers will be used throughout the drawings to represent the same parts.

### DETAILED DESCRIPTION OF THE INVENTION

The present disclosure now will be described more fully hereinafter with reference to the accompanying drawings, in which an exemplary embodiment of the disclosure is shown. This disclosure may, however, be embodied in many different forms and should not be construed as limited to the embodiments set forth herein.

Figs. 1, 3 and 4 illustrate a sectional diagram of a steam turbine 10 according to an embodiment of the disclosure. The steam turbine 10 includes a casing 12 in which a turbine rotor 13 is mounted rotatably about an axis of rotation 14. The steam turbine 10 further includes a turbine high pressure (HP) section 16 and a turbine intermediate pressure (IP) section 18. The steam turbine 10 operates at sub-critical operating conditions. In one embodiment the steam turbine 10 receives steam at a pressure below 230 bar. In another embodiment, the steam turbine 10 receives steam at a pressure between about 100 bar to about 230 bar. In another embodiment, the steam turbine 10 receives steam at a pressure between about 125 bar to 175 bar. Additionally, the steam turbine 10 receives steam at a temperature between about 525°C and about 600°C. In another embodiment, the steam turbine 10 receives steam at a temperature between about 565°C and about 600°C.

The casing 12 includes an HP casing 12a and an IP casing 12b. In another embodiment, the casing 12 may be a single, integrated HP/IP casing. In this exemplary embodiment, the casing 12 is a double wall casing. In another embodiment, the casing may be a single wall casing. The casing 12 includes a housing 20 and a plurality of guide vanes 22 attached to the housing. The rotor 13 includes a shaft 24 and a plurality of blades 25 fixed to the shaft 24. The shaft 24 is rotatably supported by a first bearing 236, a second bearing 238, and third bearing 264. In another embodiment, various bearing support configurations may be used.

A main steam flow path 26 is defined between the casing 12 and the rotor 13. The main steam flow path 26 includes a HP main steam flow path 30 located in the turbine HP section 16 and a IP main steam flow path 36 located in the turbine IP section 18. As used herein, the term "main steam flow path" means the primary flow path of steam that produces power.

Steam is provided to an HP inlet region 28 of the main steam flow path 26. The steam flows through an HP main steam flow path section 30 of the main steam flow path 26 between vanes 22 and blades 25, during which the steam expands and cools. Thermal energy of the steam is converted into mechanical, rotational energy as the steam rotates the rotor 13 about the axis 14. After flowing through the HP main steam flow path section 30, the steam flows out of an HP steam outlet region 32 into an intermediate superheater (not shown), where the steam is heated to a higher temperature. The steam is introduced via lines (not shown) to a IP steam inlet region 34. The steam flows through an IP main steam flow path section 36 of the main steam flow path 26 between vanes 22 and blades 25, during which the steam expands and cools. Additional thermal energy of the steam is converted into mechanical, rotational energy as the steam rotates the rotor 13 about the axis 14. After flowing through the IP main steam flow path section 36, the steam flows out of an IP steam outlet region 38 out of the steam turbine 10. The steam may be used in other operations, not illustrated in any more detail.

Fig. 2 illustrates a sectional view of the rotor 13. Rotor 13 includes a shaft 24. As can be seen in Fig. 2, rotor 13 includes a rotor HP section 210 located in the turbine HP section 16 (Fig. 1) and a rotor IP section 212 located in the turbine IP section 18 (Fig. 1). The shaft 24 includes a first low temperature material (LTM) section 240, a high temperature material section 242, and a second LTM section 262 Correspondingly, the shaft 24 includes a shaft HP section 220 including the first LTM section 240 and a first portion 242A of the HTM section 242 located in the turbine HP section 16 and a shaft IP section 222 including a second portion 242B of the HTM section 242 and the second LTM section 262 located in the turbine IP section 18.

The shaft HP section 220 may be joined to another component (not shown) at the first end 232 of the shaft 24 by a bolted joint, a weld, or other joining technique. In another embodiment, the shaft HP section may be bolted to a generator at the first end 232 of shaft 24. The shaft IP section 222 may be joined to another component (not shown) at a second end 234 of the shaft 24 by a bolted joint, a weld, or other joining technique. In another embodiment, the shaft IP section may be joined to a low pressure section at the second end 234 of shaft 24. In an embodiment, the low pressure section may include a low pressure turbine.

The shaft HP section 220 receives steam at a pressure below 230 bar. In another embodiment, the shaft HP section 220 may receive steam at a pressure between about 100 bar to about 230 bar. In another embodiment, the shaft HP section 220 may receive steam at a pressure between about 125 bar to about 175 bar. The shaft HP section 220 receives steam at a temperature of between about 525°C and about 600°C. In another embodiment, the shaft HP section 220 may receive steam at a temperature between about 565°C and about 600°C.

As discussed above, the shaft HP section 220 includes a first low temperature material (LTM) section 240 and a first portion 242A of the HTM section 242. The first LTM section 240 may be referred to as an HP LTM section. The shaft HP section 220 is rotatably supported by a first bearing 236 (Fig. 1) and a second bearing 238 (Fig. 1). In an embodiment, the first bearing 236 may be a journal bearing. In an embodiment, the second bearing 238 may be a thrust/journal bearing. The first bearing 236 supports the first LTM section 240, and the second bearing 238 supports the HTM section 242. In another embodiment, different support bearing configurations may be used.

The first LTM section 240 is joined to the HTM section 242 by a first weld 250. In this exemplary embodiment, the first weld 250 is located along the HP main steam flow path 30 (Fig. 3). In another embodiment, the first weld 250 may be located along the HP main steam flow path 30 where the steam temperature is less than about 455°C. In another embodiment, the first weld 250 may be located outside or not in contact with the HP steam flow path 30. In an embodiment, the first weld 250 may be located at position "A" (Fig. 1 and 2) outside and not in contact with the HP steam flow path 30, but in contact with seal steam leakage.

The HTM section 242 at least partially defines the HP main steam flow path 30 (Fig. 3). The first LTM section 240 further at least partially defines the HP main steam main flow path 30. As discussed above, in another embodiment, the weld 250 may be moved, for example to position A, so that the first LTM section 240 does not at least partially define the HP main steam flow path 30.

The HTM section 242 is formed of a single, unitary section or block of high temperature resistant material. The HTM section 242 has a first end 242a and a second end 242b. In another embodiment, the HTM section 242 may be formed of two or more HTM sections or blocks of high temperature material joined together. In an embodiment, the HTM section 242 may be formed of two or more HTM sections or blocks of high temperature material welded together.

The high temperature material may be a forging steel. In an embodiment, the high temperature material may be a steel including an amount of chromium (Cr), molybdenum (Mo), vanadium (V), and nickel (Ni). In an embodiment, the high temperature resistant material may be a high chromium alloy forged steel including Cr in an amount between about 10.0 weight percent (wt.%) to about 13.0 wt.%. In another embodiment, the amount of Cr may be included in an amount between about 10.0 wt.% and 10.6 wt.%. In an embodiment, the high chromium alloy forged steel may have Mo in an amount between 0.5 wt.% and about 2.0 wt.%. In another embodiment, the amount of Mo may be included in an amount of between 1.0 wt.% and 1.2 wt.%. In an embodiment, the high chromium alloy forged steel may include V in an amount between about 0.1 wt.% and 0.3 wt.%. In another embodiment, the V may be included in amount between about 0.15 wt.% and about 0.25 wt.%. In an embodiment, the high chromium alloy forged steel may include Ni in an amount between about 0.5 wt.% to about 1.0 wt.%. In another embodiment, the Ni may be included in an amount between about 0.6 wt.% and about 0.8 wt.%.

The first LTM section 240 is formed of a less heat resistant material than the high temperature material forming the HTM section 242. The less heat resistant material may be referred to as a low temperature material. The low temperature material may be a forged alloy steel. In an embodiment, the low temperature material may be a CrMoVNi. In an embodiment, Cr may be included in an amount between about 0.5 wt.% and about 2.2 wt.%. In another embodiment, Cr may be included in an amount between about 0.5 wt.% and about 2.0 wt.%. In another embodiment, Cr may be included in an amount between about 0.9 wt.% and about 1.3 wt.%. In an embodiment, Mo may be included in an amount between about 0.5 wt.% and about 2.0 wt.%. In another embodiment, Mo may be included in an amount between about 1.0 wt.% and about 1.5 wt.%. In an embodiment, V may be included in an amount between about 0.1 wt.% and about 0.5 wt.%. In another embodiment, V may be included in an amount of between about 0.2 wt.% and about 0.3 wt.%. In an embodiment, Ni may be included in an amount between about 0.2 wt.% to about 1.0 wt.%. In another embodiment, Ni may be included in an amount between about 0.3 wt.% and about 0.6 wt.%.

In this embodiment, the first LTM section 240 is formed of a single, unitary block or section of low temperature material. In another embodiment, the first LTM section 240 may be formed of two or more LTM sections or blocks that are joined together. The two or more LTM sections or blocks may be mechanically or materially joined together, for example, such as, but not limited to bolting or welding.

The shaft IP section 222 is rotatably supported by third bearing 264 (Fig. 1). In an embodiment, the third bearing 264 may be a journal bearing. In another embodiment, the shaft IP section 222 may be rotatably supported by one or more bearings. The shaft IP section 222 receives steam at a pressure below about 70 bar. In another embodiment, the shaft IP section 222 may receive steam at a pressure of between about 20 bar to 70 bar. In yet another embodiment, the shaft IP section 222 may receive steam at a pressure of between about 20 bar to about 40 bar. Additionally, the shaft IP section 222 receives steam at a temperature of between about 525°C and about 600°C. In another embodiment, the shaft IP section 222 may receive steam at a temperatures of between about 565°C and about 600°C.

The shaft IP section 222 includes the second portion 242B of the HTM section 242 and an second LTM section 262. The shaft HTM and second LTM sections 242, 262 are joined by a second weld 266. The second weld 266 is located along the IP steam flow path 36. In an embodiment, the second weld 266 may be located along the IP steam flow path 36 where the steam temperature is less than 455°C. In another embodiment, the second weld 266 may be located outside or not in contact with the IP steam flow path 36. For example, the second weld 266 may be located at position "B" (Fig. 1) located outside and not in contact with the IP steam flow path 36. In another embodiment, the shaft IP section 222 may include one or more HTM sections. In another embodiment, the IP section 222 may be formed of a single, unitary block or section of high temperature material.

Referring to Fig. 4, the HTM section 242 at least partially defines the IP steam inlet region 34 and IP main steam flow path 36. The second LTM section 262 further at least partially defines the IP main steam flow path 36. In another embodiment, the weld 260 may be moved, for example to position "B", so that the second LTM section 262 does not at least partially define the IP main steam flow path 36 or in other words, the second LTM section 262 is outside of the IP main steam flow path 36 and does not contact main flow path of steam.

The second LTM section 262 is formed of a less heat resistant material than the HTM section 242. The less heat resistant material section may be referred to as a low temperature material. The low temperature material may be a low temperature material as discussed above in reference to the first LTM section 240. In this embodiment, the second LTM section 262 is formed of a single, unitary section or block of low temperature material. In another embodiment, the second LTM section 262 may be formed of two or more LTM sections that are joined together. The two or more LTM sections may be mechanically or materially joined together, for example, such as, but not limited to bolting or welding. In an embodiment, the second LTM section 262 is formed of the same low temperature material as the first LTM section 240. In another embodiment, the second LTM section 240 is formed of different low temperature material as the first LTM section 240.

Fig. 5 illustrates another embodiment of a steam turbine 500 according to the present disclosure. As can be seen in Fig. 5, which is a simplified illustration of the embodiment for viewing purpose, the steam turbine 500 includes a casing 512, in which a rotor 513 is mounted rotatably about an axis of rotation 514. The steam turbine 500 includes a turbine high pressure (HP) section 516 and a turbine intermediate pressure (IP) section 518. The steam turbine 500 operates at sub-critical operating conditions. In one embodiment the steam turbine 500 receives steam at a pressure below 230 bar. In another embodiment, the steam turbine 500 receives steam at a pressure between about 100 bar to about 230 bar. In another embodiment, the steam turbine 500 receives steam at a pressure between about 125 bar to about 175 bar. Additionally, the steam turbine 500 receives steam at a temperature between about 525°C and about 600°C. In another embodiment, the steam turbine 500 receives steam at a temperature between about 565°C and about 600°C.

The casing 512 includes an HP casing portion 512a and an IP casing portion 512b. The casing 512 is a single wall, integrated HP/IP casing. The casing 512 may be referred to as a housing. In another embodiment, the casing 512 may be two or more casings, such as, but limited to the two part casing 12 (Fig. 1) discussed above. The casing 512 includes a plurality of guide vanes 522 fixed thereto.

The rotor 513 includes a shaft 524 and a plurality of blades 525 fixed to the shaft 524. A main steam flow path 526 is defined between the casing 512 and the rotor 513. The main steam flow path 526 includes a HP main steam flow path 530 located in the turbine HP section 516 and a IP main steam flow path 536 located in the turbine IP section 518. As used herein, the term "main steam flow path" means the primary flow path of steam that produces power.

Steam is provided to an HP inlet region 528 of the main steam flow path 526. The steam flows through an HP main steam flow path section 530 of the main steam flow path 526 between vanes 522 and blades 525, during which the steam expands and cools. Thermal energy of the steam is converted into mechanical, rotational energy as the steam rotates the rotor 513 about the axis 514. After flowing through the HP main steam flow path section 530, the steam flows out of an HP steam outlet region 532 into an intermediate superheater (not shown), where the steam is heated to a higher temperature. The steam is introduced via lines (not shown) to a IP steam inlet region 534. The steam flows through an IP main steam flow path section 536 of the main steam flow path 526 between vanes 522 and blades 525, during which the steam expands and cools. Additional thermal energy of the steam is converted into mechanical, rotational energy as the steam rotates the rotor 513 about the axis 514. After flowing through the IP main steam flow path section 536, the steam flows out of an IP steam outlet region 538 out of the steam turbine 500. The steam may be used in other operations, not illustrated in any more detail.

The rotor 513 includes a rotor HP section 610 located in the turbine HP section 516 and a rotor IP section 612 located in the turbine IP section 618. Correspondingly, the shaft 524 includes a shaft HP section 620 located in the rotor HP section 610 and a shaft IP section 622 located in the rotor IP section 612. A section divider 638 is a stationary sealing structure that separates the HP steam inlet region 528 from the IP steam inlet region 534.

The shaft HP section 620 may be joined to another component (not shown) at the first end 632 of the shaft 524 by a bolted joint, a weld, or other joining technique. In another embodiment, the shaft HP section 620 may be bolted to a generator at the first end 632. The shaft IP section 622 may be joined to another component (not shown) at a second end 634 of the shaft 524 by a bolted joint, a weld, or other joining technique. In another embodiment, the shaft IP section 622 may be joined at the second end 634 to a low pressure section that may include a low pressure turbine.

The shaft HP section 620 receives steam at a pressure below 230 bar. In another embodiment, the shaft HP section 620 may receive steam at a pressure between about 100 bar to about 230 bar. In another embodiment, the shaft HP section 620 may receive steam at a pressure between about 125 bar to about 175 bar. The shaft HP section 620 receives steam at a temperature of between about 525°C and about 600°C. In another embodiment, the shaft HP section 620 may receive steam at a temperature between about 565°C and about 600°C.

The shaft HP section 620 includes a first low temperature material (LTM) section 640 and a first portion 642A of a high temperature material (HTM) section 642. The first LTM section 640 may be referred to as an HP LTM section. The shaft HP section 620 is rotatably supported by the first bearing 636. In an embodiment, the first bearing 636 may be a journal bearing or a combined thrust/journal bearing. The first bearing 636 supports the first LTM section 640. In another embodiment, different support bearing configurations may be used.

The first LTM section 640 is joined to the HTM section 642 by a first weld 650. In this exemplary embodiment, the first weld 650 is located along the HP main steam flow path 530. In another embodiment, the first weld 650 may be located along the HP main steam flow path 530 where the steam temperature is less than 455°C. In another embodiment, the first weld 650 may be located outside or not in contact with the HP steam flow path 530. In an embodiment, the first weld 650 may be located at position "A" outside and not in contact with the HP steam flow path 530, but in contact with seal steam leakage.

The HTM section 642 at least partially defines the HP main steam flow path 530. The first LTM section 640 further at least partially defines the HP main steam main flow path 530. As discussed above, in another embodiment, the first weld 650 may be moved, for example to position A, so that the first LTM section 640 does not at least partially define the HP main steam flow path 530.

The HTM section 642 of the shaft 24 is formed of a single, unitary section or block of high temperature material. The HTM section 642 has a first end 642a and a second end 642b. In another embodiment, the HTM section 642 may be formed of two or more HTM sections or blocks of high temperature material that are joined together by a material joining technique, such as, but not limited to welding.

The high temperature material may be a forging steel. In an embodiment, the high temperature material may be a steel including an amount of chromium (Cr), molybdenum (Mo), vanadium (V), and nickel (Ni). In an embodiment, the high temperature material may be a high chromium alloy forged steel including Cr in an amount between about 10.0 weight percent (wt.%) to about 13.0 wt.%. In another embodiment, the amount of Cr may be included in an amount between about 10.0 wt.% and about 10.6 wt.%. In an embodiment, the high chromium alloy forged steel may have Mo in an amount between about 0.5 wt.% and about 2.0 wt.%. In another embodiment, the amount of Mo may be included in an amount of between about 1.0 wt.% and about 1.2 wt.%. In an embodiment, the high chromium alloy forged steel may include V in an amount between about 0.1 wt.% and about 0.3 wt.%. In another embodiment, the V may be included in amount between about 0.15 wt.% and about 0.25 wt.%. In an embodiment, the high chromium alloy forged steel may include Ni in an amount between about 0.5 wt.% to about 1.0 wt.%. In another embodiment, the Ni may be included in an amount between about 0.6 wt.% and about 0.8 wt.%.

The first LTM section 640 is formed of a less heat resistant material than the high temperature material forming the HTM section 642. The less heat resistant material may be referred to as a low temperature material. The low temperature material may be a forged alloy steel. In an embodiment, the low temperature material may be a CrMoVNi. In an embodiment, Cr may be included in an amount between about 0.5 wt.% and about 2.2 wt.%. In another embodiment, Cr may be included in an amount between about 0.5 wt.% and about 2.0 wt.%. In another embodiment, Cr may be included in an amount between about 0.9 wt.% and about 1.3 wt.%. In an embodiment, Mo may be included in an amount between about 0.5 wt.% and about 2.0 wt.%. In another embodiment, Mo may be included in an amount between about 1.0 wt.% and about 1.5 wt.%. In an embodiment, V may be included in an amount between about 0.1 wt.% and about 0.5 wt.%. In another embodiment, V may be included in an amount of between about 0.2 wt.% and about 0.3 wt.%. In an embodiment, Ni may be included in an amount between about 0.2 wt.% to about 1.0 wt.%. In another embodiment, Ni may be included in an amount between about 0.3 wt.% and about 0.6 wt.%.

In this embodiment, the first LTM section 640 is formed of a single, unitary block or section of low temperature material. In another embodiment, the first LTM section 640 may be formed of two or more LTM sections or blocks that are joined together. The two or more LTM sections or blocks may be mechanically or materially joined together, for example, such as, but not limited to bolting or welding.

The shaft IP section 622 is rotatably supported by the second bearing 664. In an embodiment, the second bearing 664 may be a journal bearing or a combined thrust/journal bearing. In another embodiment, the shaft IP section 622 may be rotatably supported by one or more bearings.

The shaft IP section 622 receives steam at a pressure below about 70 bar. In another embodiment, the shaft IP section 622 may receive steam at a pressure of between about 20 bar to 70 bar. In yet another embodiment, the shaft IP section 622 may receive steam at a pressure of between about 20 bar to about 40 bar. Additionally, the shaft IP section 622 receives steam at a temperature of between about 525°C and about 600°C. In another embodiment, the shaft IP section 622 may receive steam at a temperatures of between about 565°C and about 600°C.

The shaft IP section 622 includes a second portion 642B of the HTM section 642 and an second LTM section 662. The shaft HTM and second LTM sections 642, 662 are joined by a second weld 666. The second weld 666 is located along the IP steam flow path 536. In another embodiment, the second weld 666 may be located along the IP steam flow path 536 where the steam temperature is less than about 455°C. In another embodiment, the second weld 666 may be located outside or not in contact with the IP steam flow path 536. For example, the second weld 666 may be located at position "B" located outside and not in contact with the IP steam flow path 536. In another embodiment, the shaft IP section 622 may include one or more HTM sections. In another embodiment, the IP section 622 may be formed of a single, unitary block or section of high temperature material.

The HTM section 642 at least partially defines the IP steam inlet region 534 and IP main steam flow path 536. The IP LTM section 662 further at least partially defines the IP main steam flow path 536. In another embodiment, the second weld 666 may be moved, for example to position "B", so that the IP LTM section 662 does not at least partially define the IP main steam flow path 536 or in other words, the IP LTM section 662 is outside of the IP main steam flow path 536 and does not contact main flow path of steam.

The second LTM section 662 is formed of a less heat resistant material than the HTM section 642. The less heat resistant material section may be referred to as a low temperature material. The low temperature material may be a low temperature material as discussed above in reference to the first LTM sections 640. In this embodiment, the second LTM section 662 is formed of a single, unitary section or block of low temperature material. In another embodiment, the second LTM section 662 may be formed of two or more LTM sections that are joined together. The two or more LTM sections may be mechanically or materially joined together, for example, such as, but not limited to bolting or welding. In an embodiment, the second LTM section 662 is formed of the same low temperature material as the first LTM section 640. In another embodiment, the second LTM section 640 is formed of different low temperature material as the first LTM section 640.

The shaft 524 may be produced by an embodiment of a method of manufacturing as described below. The shaft 524 may be produced by providing a block or section of a high temperature material that forms the HTM section 642 having a first end 642a and a second end 642b. A first LTM section 640 formed of a block or section of a low temperature material is welded to the first end 642a of the HTM section 642. In another embodiment, the shaft 524 may be produced by providing one or more blocks or sections of a high temperature material that forms the HTM section 642 having a first end 242a and a second end 242b and welding a first LTM section 640 formed of one or more blocks of low temperature material to the first end 642a of the HTM section 642. The shaft 524 is further produced by welding a second LTM section 662 to a second end 642b of the HTM section 642. In another embodiment, a shaft 524 may be produced by welding one or more blocks of low temperature material that forms the second LTM section 662 to the second end 642b of the HTM section 642.

While only certain features and embodiments of the invention have been shown and described, many modifications and changes may occur to those skilled in the art (for example, variations in sizes, dimensions, structures, shapes and proportions of the various elements, values of parameters (for example, temperatures, pressures, etc.), mounting arrangements, use of materials, colors, orientations, etc.) without materially departing from the novel teachings and advantages of the subject matter recited in the claims. The order or sequence of any process or method steps may be varied or re-sequenced according to alternative embodiments. It is, therefore, to be understood that the appended claims are intended to cover all such modifications and changes as fall within the true scope of the invention. Furthermore, in an effort to provide a concise description of the exemplary embodiments, all features of an actual implementation may not have been described (i.e., those unrelated to the presently contemplated best mode of carrying out the invention, or those unrelated to enabling the claimed invention). It should be appreciated that in the development of any such actual implementation, as in any engineering or design project, numerous implementation specific decisions may be made. Such a development effort might be complex and time consuming, but would nevertheless be a routine undertaking of design, fabrication, and manufacture for those of ordinary skill having the benefit of this disclosure, without undue experimentation.

## Claims

1. A subcritical rotor, comprising:
a high temperature material section formed of a high temperature material;
a first low temperature material section formed of a first low temperature material attached to a first end of the high temperature material section (242);
a second low temperature material section formed of second low temperature material joined to a second end of the high temperature material section (242);
wherein the high temperature material section is exposed to steam at less than 230 bar.

2. The subcritical rotor of claim 1, wherein the high temperature material section is exposed to steam between about 100 bar and less than 230 bar.

3. The subcritical rotor of claim 1 or claim 2, wherein the high temperature material is a high chromium alloy forged steel.

4. The subcritical rotor of claim 3, wherein the high chromium alloy forged steel comprises:
about 10.0 wt.% to about 13.0 wt.% Cr;
about 0.5 wt. % to about 2.0 wt. % Mo;
about 0.1 wt.% to about 0.3 wt.% V; and
about 0.5 wt. % to about 1.0 wt. % Ni.

5. The subcritical rotor of any preceding claim, wherein the low temperature material is a forged alloy steel.

6. The subcritical rotor of claim 5, wherein the forged alloy steel comprises:
about 0.5 wt.% to about 2.2 wt.% Cr;
about 0.5 wt. % to about 2.0 wt. % Mo;
about 0.1 wt.% to about 0.5 wt.% V; and
about 0.2 wt.% to about 1.0 wt.% Ni.

7. The steam turbine, comprising:
the subcritical rotor of any preceding claim.

8. The steam turbine of claim 7, further comprising:
a single wall casing.

9. A method of manufacturing a subcritical rotor of any one of claims 1 to 6 comprising:
providing a high temperature material section; and
joining a first low temperature material section to a first end of the high temperature material section; and
joining a second low temperature material section to a second end of the high temperature material section;
wherein the high temperature material section is exposed to steam at less than 230 bar.

10. The method of claim 9, wherein the high temperature material section is joined to the first and second low material sections by welding.
